

April 12, 1932.

J. O. BETTERTON

1,853,541

LIQUATION OF METALS

Filed Feb. 5, 1932



INVENTOR  
Jesse O. Betterton  
BY  
Austin & Dix  
ATTORNEYS

## UNITED STATES PATENT OFFICE

JESSE O. BETTERTON, OF METUCHEN, NEW JERSEY, ASSIGNOR TO AMERICAN SMELTING AND REFINING COMPANY, OF NEW YORK, N. Y., A CORPORATION OF NEW JERSEY

## LIQUATION OF METALS

Application filed February 5, 1932. Serial No. 591,197.

This invention relates to the refining of metals, and more particularly to the removal and recovery of bismuth from various metals in which it may be present as an impurity, 5 as for example, from lead bullion.

The present invention provides for removing the bismuth from the lead bullion in combination with certain other impurities in a 10 complex dross and then treating the dross by liquation for the selective removal of the various metals therefrom.

The invention further consists in the new and novel features of operation and the new and original arrangements and combinations 15 of steps in the process hereinafter described and more particularly set forth in the claims.

Although the novel features which are believed to be characteristic of this invention will be particularly pointed out in the claims, 20 appended hereto, the invention itself, as to its objects and advantages, the mode of its operation and the manner of its organization may be better understood by referring to the following description taken in connection with the accompanying drawing forming a part 25 thereof, in which the figure is a flow sheet illustrating the present process.

In the following description and in the claims the various steps in the process and the 30 details comprising the invention will be identified by specific names for convenience but they are intended to be as generic in their application as the art will permit.

The present process is carried out for the 35 removal and recovery of bismuth from lead bullion by suitably treating the bullion as by the addition of zinc to remove the silver therefrom as a zinc-silver dross, and thereafter applying to the bath of molten lead a suitable 40 reagent, such as an alkali earth metal, preferably alloyed with lead or lead with some zinc to form a dross containing the bismuth, the alkali earth metal, zinc and lead. This 45 dross is then removed from the bath and melted under a suitable cover slag after which the lead is removed by liquation and the alkali earth metal and bismuth are separated from the cover slag by selective tapping and are treated for the recovery of the metal values.

More specifically the invention may be car-

ried out by adding to the lead bullion zinc and blocks containing some silver from previous refining operations and bringing the bath to a temperature of 870° F. to 900° F. while the bath is suitably stirred to produce the desired 55 reaction. A zinc-silver dross then forms on the surface of the bath which may be pressed to largely separate the lead therefrom and may be removed from the bath. The dross is then treated in retorts wherein the silver is 60 recovered in the usual manner.

After the dross has been removed zinc plates may be added and the bath gradually allowed to cool to a temperature of 660° F. 65 while further quantities of dross are formed and simultaneously removed. This dross may be cast into blocks and returned to the bullion as above mentioned as a source of zinc in the desilverizing step.

Thereupon a suitable alkali earth metal, 70 such for example as calcium, preferably in the form of a lead alloy or in the form of a lead-zinc alloy is added to the bath. At the same time blocks and rims, together with lead and zinc containing all of the alkaline metal, 75 plus silver from subsequent steps of the process, to be hereinafter described, are added to the bath. The bath is then vigorously stirred, preferably by a mechanical stirrer, and at this stage of the operation the bath is carefully held at a temperature of 640 to 80 660° F. at which temperatures oxidation of the calcium is almost completely prevented and also a much higher ratio of bismuth extraction per pound of calcium is secured. 85 The resulting dross which comprises bismuth, calcium, zinc, lead and some silver may then be pressed, if desired, to reduce the lead content and removed from the bath and further treated for the recovery of the metal values 90 in the manner to be described.

Thereafter, the bath may be cooled to about 625° F. and blocks may be formed from the resulting dross. Rims may be also formed 95 adjacent the sides of the container as the metal solidifies. These blocks and rims may be returned to the bath as above described.

The zinc and calcium are now removed from the bath by reheating the same to a temperature of 670° F. to 750° F. and adding a 100

zinc chloride cover thereto in sufficient quantity to completely cover the top of the bath. Chlorine is introduced into the bath beneath this cover and unites with the zinc and calcium to form slags of zinc chloride and calcium chloride. The first slag formed will contain all of the calcium as calcium chloride and some of the zinc as zinc chloride. This may be removed and used in any suitable manner or may be discarded. The final slag which is formed after calcium is removed represents the normal zinc chloride salt and may be used as such. The lead bath after the removal of the above impurities may be further refined in any well known manner.

The bismuth-calcium-zinc-lead-silver dross above mentioned which has been removed from the lead bath is then heated under a cover slag of calcium chloride together with sodium chloride which has preferably been dehydrated. One method of carrying out this step is to heat the calcium chloride mixed with sodium chloride in a suitable kettle to a temperature of 1000°-1300° F., add the above mentioned dross and heat the mixture to a temperature sufficient to substantially melt the contents of the kettle, for example, a temperature of 1000°-1300° F.

The bath is then cooled sufficiently to solidify both the slag and a crust composed of calcium, bismuth and a large part of the zinc which forms immediately beneath the solidified slag, but the bath is not cooled sufficiently to freeze the lead and the remainder of the zinc. Temperatures of 800° F. to 900° F. have been found suitable for this purpose. The lead and zinc containing silver but only a small amount of bismuth and calcium is then tapped and returned to the lead bullion, together with the calcium-lead alloy ahead of the debismuthizing step as previously described.

The kettle containing the slag and the calcium-bismuth-zinc layer is then reheated to a temperature sufficient to substantially melt the same, as for example, 1000° F. to 1800° F. and the calcium-bismuth-zinc layer is tapped and suitably treated to separate and recover the calcium, bismuth and zinc therefrom. This layer contains a relatively small amount of lead, for example 10 to 30%, and calcium in amounts of approximately one-half to one-third of the bismuth content.

The molten slag of calcium chloride and sodium chloride which may contain small quantities of calcium oxide is then tapped or otherwise removed from the kettle and sent to a suitable recovery apparatus or discarded.

By means of my improved process the removal of bismuth is carried out in combination with the usual desilverizing steps, thereby saving time and labor involved in twice cooling the bath almost to the melting point of lead, and also saving the expense and labor involved in re-heating the kettle to a rela-

tively high temperature intermediate of two cooling steps.

Not only is the bismuth removed almost completely, but a substantial amount of zinc usually remaining in lead bullion after the desilverizing step is also removed and may be recovered as metallic zinc with the resulting economy in the cost of the operation. For example, the zinc which remains as the eutectic with lead amounts to approximately .56% after desilverization but by my process the amount of zinc remaining is reduced to approximately .3% which results in a saving of approximately 40% of the zinc that previously was drossed off and then in the subsequent operations was lost in the slag. Furthermore, the zinc and calcium which are used in the above steps as reagents are removed simultaneously from the lead bath and duplication of operations is thus avoided. The process has been described as carried out by the use of a calcium-lead alloy or the use of a calcium-lead-zinc alloy for the removal of bismuth but it is to be understood that other alkali earth metals including magnesium may be substituted for the calcium and may be removed from the lead bath and from the bismuth dross in a corresponding manner.

Although certain novel features of the invention have been shown and described and are pointed out in the annexed claims, it will be understood that various omissions, substitutions and changes in the several steps of the process and in its operation may be made by those skilled in the art without departing from the spirit of the invention.

The present application is a continuation in part of Betterton, Serial Number 492,852, filed November 1, 1930.

What is claimed is:

1. The process of removing impurities, such as silver, zinc and bismuth, from lead bullion which comprises removing silver as a zinc-silver dross, removing the bismuth and a portion of the residual zinc by the addition of an alkali earth metal as a dross, melting said dross under a cover slag, separating the lead therefrom by liquation and separating the bismuth and alkali earth metal from the cover slag by selective tapping.

2. The process of removing bismuth from lead which comprises adding to a bath of molten lead a reagent yielding an alkali earth metal within the body of the molten lead in a condition capable of forming a dross with said bismuth, removing said dross and melting the same under a chloride slag, separating the lead from said dross by liquation and returning the lead to the original lead bath ahead of the debismuthizing step, heating the liquate to cause the slag and the bismuth to separate into different layers and selectively removing said layers.

3. The process of recovering bismuth

from lead containing bismuth as an impurity which comprises adding a calcium alloy to a bath of molten lead under conditions suitable for the formation of a calcium-bismuth-lead dross, removing said dross from the bath, melting the same under a chloride slag, separating the lead from the dross by liquation, causing the calcium and bismuth to separate from the slag as a distinct layer and 10 removing said layer.

4. The process of recovering bismuth from a mixture containing bismuth, calcium and lead which comprises melting said mixture under a chloride slag, cooling to a temperature at which the slag and a layer of calcium and bismuth separate from the lead and solidify, removing the molten lead therefrom, reheating to completely fuse the slag, calcium and bismuth and to cause them to maintain distinct layers and separately removing 20 said layers by selective tapping.

5. The process of separating bismuth, calcium and lead from mixtures containing these metals which comprises melting said mixture under a slag of calcium chloride and sodium chloride, heating the mixture to a temperature at which all of the constituents are molten, cooling the mixture to a temperature at which the slag and the calcium and bismuth solidify while the lead remains molten, removing the molten lead, reheating the mixture to a temperature at which all of the remaining constituents are molten, allowing said constituents to separate in two 30 layers, one layer containing the calcium chloride and sodium chloride, and the other layer containing the calcium and bismuth, separating said layers and treating the calcium-bismuth layer for the recovery of bismuth.

6. The process of separating bismuth, calcium and lead from mixtures thereof which comprises heating said mixture under a layer of calcium chloride and sodium chloride to a temperature of 1000° F. to 1300° F., cooling the mixture to a temperature of 800° F. to 900° F. whereby the lead is separated by liquation, removing the molten lead, reheating the remaining constituents to a temperature 45 of 1000° F. to 1800° F. whereby the calcium chloride and sodium chloride separate as one layer and the calcium and bismuth as a second layer, removing the layer of calcium and bismuth and treating the same for the recovery of said metals.

7. The process of removing impurities, such as bismuth and silver, from lead which comprises adding zinc to a bath of molten lead and removing the resultant zinc-silver dross, adding an alkali earth metal to said bath and removing the resultant dross containing bismuth, treating the bath under a chloride slag with chlorine gas to remove the zinc and alkali earth metal as chlorides and treating the 55 bismuth dross by melting said dross under

a chloride slag, liquating the same to separate lead, returning the lead so separated to the original bath ahead of the debismuthizing step, causing the bismuth and alkali earth metal to separate as a distinct layer from the 70 chloride slag and separately removing said layer and treating the same for the recovery of bismuth therefrom.

8. The process of recovering bismuth from a lead bath containing this element as an impurity which comprises adding calcium to said bath and allowing a bismuth-calcium-lead dross to form, removing said dross, treating the bath with chlorine under conditions favorable to the formation of a calcium chloride slag, whereby the calcium is removed therefrom, separately treating the bismuth dross by melting under a chloride slag, separating the lead therefrom by liquation and separating the calcium and bismuth from said 85 slag by heating the mixture to substantially liquefy the various constituents, whereby the calcium and bismuth separate as a distinct layer.

9. The process of removing bismuth from lead containing the same as an impurity which comprises treating a bath of said lead with a reagent yielding an alkali earth metal within the body of the molten lead in a condition capable of forming a dross containing 90 said bismuth, removing the dross and melting the same under a chloride slag, separating the lead from said dross by liquation and returning the lead to the original bath, and separating the bismuth from the slag by heating the mixture to a temperature at which the various constituents become liquid, whereby the slag forms a layer above the bismuth and may be mechanically separated therefrom.

10. The process of recovering bismuth from a lead bath containing the same as an impurity which comprises treating said bath with a reagent yielding an alkali earth metal within the body of the molten lead in a condition capable of forming a dross containing bismuth, removing said dross from the bath, melting said dross under a cover slag and cooling to a temperature at which the slag and the bismuth solidify and the lead remains molten, removing the molten lead and returning the same to the original bath, reheating the dross to a temperature at which all of the constituents become molten, allowing the bismuth to separate as a distinct layer 115 from the slag and mechanically separating said layers.

In testimony whereof I have hereunto set my hand.

JESSE O. BETTERTON. 125